

# UNITED STATES PATENT OFFICE.

CHARLES N. FORREST, OF RAHWAY, AND JOSEPH V. MEIGGS, OF PERTH AMBOY, NEW JERSEY, ASSIGNORS TO THE BARBER ASPHALT PAVING COMPANY, OF PHILADELPHIA, PENNSYLVANIA, A CORPORATION OF WEST VIRGINIA.

## MANUFACTURE OF RESINOUS PRODUCTS.

1,305,790.

Specification of Letters Patent.

Patented June 3, 1919.

No Drawing.

Application filed December 31, 1917. Serial No. 209,706.

*To all whom it may concern:*

Be it known that we, CHARLES N. FORREST and JOSEPH V. MEIGGS, citizens of the United States of America, residing in Rahway, county of Union, and State of New Jersey, and Perth Amboy, county of Middlesex, and State of New Jersey, respectively, have invented certain new and useful Improvements in the Manufacture of Resinous Products, 10 of which the following is a specification.

The object of our invention is to provide balsamic and resinous products by the action of nitric acid upon the unsaturated hydrocarbons of the distillates from petroleum or from the native solid bitumens.

All such distillates are composed of both saturated and unsaturated hydrocarbons and as a means of differentiating between these 20 two classes of substances they may be treated with sulfuric acid, first with ordinary 66° acid and finally with fuming sulfuric acid. That portion which is unacted upon by such acid treatment consists of the saturated hydrocarbons and that portion which is acted upon constitutes the unsaturated hydrocarbons as referred to in this specification. It is this unsaturated portion which is the source of the materials we have discovered. The unsaturated portion consists of olefins, naphthenes, polymethylenes, and the sulfur, nitrogen and oxygen derivatives thereof, while the saturated portion consists of liquid paraffins. It is not desirable to select for this purpose any distillates which are composed largely of saturated paraffin hydrocarbons and we preferably select that distillate which contains the highest amount of unsaturated bodies. It is found that the 40 distillates obtained by the destructive distillation of asphaltic petroleum or of the solid asphalts are preferable for our purpose and the distillate obtained in the destructive distillation of gilsonite is especially desirable. We will therefore confine our illustration of our method for the production of these substances to the distillates from the destructive distillation of gilsonite. Such distillates may be obtained by any of 50 the methods of distillation in common use

for destructively distilling oils, as the desirability of any distillate for our purpose is inherent in the original substance rather than being due to the particular method by which it is distilled in the first instance.

While the treatment of the liquid hydrocarbons with sulfuric acid, as hereinbefore described, will differentiate between the saturated and unsaturated hydrocarbons, it is not desirable to isolate the latter class of 60 hydrocarbons by such means for the purpose of this invention. In fact it is most undesirable to do so because the sulfuric acid treatment carbonizes the oil and also produces sulfonic bodies which are undesirable for our purpose. On the contrary we proceed with the mixed hydrocarbons, since those of the saturated class are inert and can be separated from our new product after it is formed by our process from the unsaturated hydrocarbons in the presence of 70 the saturated hydrocarbons.

It is to be understood that such distillates have a wide range of boiling points, say from 150° F. to 700° F. and while it is sometimes desirable to proceed with such a combination of substances it is generally more desirable to select some fraction or combination of fractions thereof, say that below 400° F. or between 400° F. and 600° 80 F. or even narrower fractions, say between 550 and 600° F. We may also select specific fractions and recombine them in new proportions and thereby obtain superior results.

This is because the material produced from the lower boiling fraction is softer than that produced from the higher fractions, and the selection of the proper fraction permits of the possibility of producing products varying in hardness from a soft balsam like material to a hard resin. In general, however, it is intended to produce three grades which are respectively soft, medium and hard, all of which are of light 90 color and are completely soluble in methyl, ethyl and higher alcohols, acetone and the higher ketones, while at the same time they are insoluble or virtually so in petroleum ether and in carbon disulfid.

55

65

70

75

80

85

90

95

100

Our new products are also insoluble in water and dilute mineral acids. They are softened slightly by moderate heat, say below 212° F. and intumesce and carbonize 5 rather than melt at temperatures at which common resin (colophony) asphalt and similar substances safely melt.

The special utility of our products lies in their capacity to combine or mix with pyroxylin in all proportions in the presence of 10 a mutual solvent and the consequent utilization of such mixtures as lacquer, leather dressings and in the production of artificial leather, which usually consist of a coating 15 of nitro-cellulose products and nitrated vegetable oils on woven or felted fabrics. They are also a substitute for shellac in many, if not all, commercial applications, especially if some pyroxylin be added.

20 In preparing our new products we select a suitable fraction or combination of fractions of the distillate from gilsonite and place it in an iron, stoneware or other vessel immune to nitric acid, which vessel is 25 provided with a jacket through which steam or hot water may be circulated for heating purposes, or cold water for cooling purposes, and then adjust the temperature of the oil to about 200° F.

30 To the oil is then added slowly in small increments, dilute nitric acid (e. g. 43° B.) while the oil is stirred in any convenient way to assist mixing. The volume of acid dropped at any one time upon the oil should 35 not exceed the ratio of 1 to 2500, and may advantageously be less, as the reaction is an exothermic one and may proceed with considerable violence if not handled cautiously. The concentration of nitric acid employed 40 may be varied to adapt itself to the nature of the particular hydrocarbons or fractions thereof under treatment and may contain from 5 to 10% HNO<sub>3</sub> up to the possible maximum.

45 The addition of acid to oil causes a rise in temperature. This should not be allowed to exceed say 200° F. Any desired temperature between 200° F. and 220° F. may be maintained by regulating the rate of 50 addition of acid to oil. However, we have found it advantageous to add the acid to the oil so slowly that the heat of reaction is wholly or almost wholly dissipated, the desired temperature (200° F.-220° F.,) being 55 maintained by the application of heat from the outside. The reaction is stopped, i. e. no more acid added, when approximately 100 parts by volume of acid have been added to 200 parts by weight of oil. The main 60 reaction product, where fractions between 400° and 600° F. are employed is a light yellow plastic semi-solid resin.

If, instead of using the fraction of gilsonite distillate below 600° F., higher fractions 65 be used, for example, a suitable distillate

above 600° F., then the reaction product on purification and drying, is a hard, solid resin.

Or, a very viscous oil, with properties closely resembling those of nitrated castor 70 oil, may be obtained by substituting in the above treatment the 0-400° F. fraction from gilsonite.

Thus, three or more grades of products 75 may be obtained from the various fractions of the gilsonite distillate, and the same statement holds good with distillates of other bitumens.

We have found the above process may be assisted, or, in fact, carried out by blowing 80 oxids of nitrogen through the oils in question, but we prefer to use nitric acid in the manner shown.

After the reaction is completed, the reaction mixture is cooled to 50°-75° F., when 85 the resinous matter separates and may be removed, or the reaction mixture may be poured into cold water and the products separated in this way. In any case, the resulting resinous mass is removed and agitated 90 thoroughly with hot water using several fresh wash waters, in order to remove free nitric acid and soluble and emulsifiable impurities. This washing is preferably assisted by the addition to the wash waters, of 95 very small amounts of ammonia, or sodium carbonate, or of chalk in suspension, afterward washing entirely free of these substances.

We also prefer in the case of products obtained from gilsonite fractions above 600° F. to further use an extremely dilute hot solution of sodium or potassium bichromate as wash water. This reagent also seems to impart a slight increased degree of solidity to 100 the resin. We take care to remove this reagent by thorough washing with hot water.

When handling a product obtained by the action of nitric acid, as above, on distillates below say 600° F., then we use a stronger 110 solution of sodium or potassium bichromate than we use in the case of the products prepared from the fractions of the gilsonite distillate above 600° F. To be specific we may use in the latter case seven (7) parts 115 e. g. Na<sub>2</sub>Cr<sub>2</sub>O<sub>7</sub> to 10000 of water and fourteen (14) parts HCl (sp. gr. 1.2). In the former case we use a 10-20% solution of Na<sub>2</sub>Cr<sub>2</sub>O<sub>7</sub> containing 2-10% HCl (sp. gr. 1.20). The use of this increased concentration of Na<sub>2</sub>Cr<sub>2</sub>O<sub>7</sub> in the former case exerts a bleaching action on the resin and renders it pale yellow. Thorough washing with hot water is then employed to remove all traces 120 of bichromate and acid. The material is 125 then dried.

When proceeding with the distillate from gilsonite, which contains not more than 25% of saturated hydrocarbons, the yield of our product by the method described amounts to

60% by weight. This rate of production is reduced to 35% from the lower boiling fractions, say from 0 to 400° F., and increased to as much as 70 to 80% from the 500 to 600° F. fractions.

5 We are aware that it has been proposed to add to hydrocarbon distillates, a mixture of nitric and sulfuric acid, until the acid mixture amounts to three parts added to one 10 part of petroleum distillate. Such process differs from that here described, in that the resulting product is solid, or semi-solid, while our products range from soft to hard, the softer products resembling molasses in 15 consistency. Again our products are virtually insoluble in petroleum ether, and in carbon disulfid, while the products of the process just named are thus soluble, a distinction which is particularly useful when 20 our products are used as a substitute for shellac.

Having thus described our invention, we claim:

25 1. The process of obtaining balsamic and resinous materials which consists in slowly and gradually adding nitric acid (or oxids of nitrogen derived therefrom) to distillates of native bitumens which contain a relatively high proportion of unsaturated and reactive liquid hydrocarbons the quantity of acid added being considerably less than the 30 quantity of distillate and separating the balsamic resinous materials thus formed from the residual liquid product.

35 2. The process of obtaining balsamic and

Copies of this patent may be obtained for five cents each, by addressing the "Commissioner of Patents, Washington, D. C."

resinous materials which consists in adding nitric acid (or oxids of nitrogen derived therefrom) to distillates of native bitumens which contain a relatively high proportion of unsaturated and reactive liquid hydrocarbons; separating the balsamic and resinous materials thus formed from the residual liquid product; and treating with a soluble bichromate to harden and bleach the product.

40 3. The process of obtaining balsamic and resinous materials which consists in adding nitric acid very slowly to distillates of native bitumens with maintenance of a temperature between 200° F. and 220° F., and with agitation and thorough mixing, and then separating the bituminous and resinous materials thus formed from the residual liquid product.

45 4. A balsamic or resinous material resulting from the reaction of nitric acid or oxids of nitrogen derived therefrom upon the unsaturated and reactive distillates of native bitumens, characterized by being soluble in alcohol and acetone, but insoluble in petroleum ether or carbon disulfid.

50 In testimony whereof, we have hereunto signed our names at Philadelphia, Pennsylvania, this twenty-eighth day of December, 1917.

CHARLES N. FORREST.  
JOSEPH V. MEIGS.

Witnesses:

JAMES H. BELL,  
E. L. FULLERTON.

1251-31